

# United States Patent [19]

Sakaguchi et al.

[11] 3,904,410

[45] Sept. 9, 1975

[54] **ELECTROPHOTOGRAPHIC COPYING PAPER**

[75] Inventors: **Kahei Sakaguchi; Noboru Moriyama; Hirotaka Takemoto**, all of Wakayama, Japan

[73] Assignee: **Kao Soap Co., Ltd.**, Tokyo, Japan

[22] Filed: **Dec. 10, 1973**

[21] Appl. No.: **423,112**

[30] **Foreign Application Priority Data**

Dec. 19, 1972 Japan..... 47-127473

[52] **U.S. Cl.** ..... 96/1.5; 96/1.7; 117/155 L; 117/201

[51] **Int. Cl.** ..... G03g 5/04

[58] **Field of Search** ..... 117/155 L, 154; 96/1.7, 96/1.5

*Primary Examiner*—Norman G. Torchin  
*Assistant Examiner*—John L. Goodrow  
*Attorney, Agent, or Firm*—Woodhams, Blanchard & Flynn

[57] **ABSTRACT**

Electrophotographic copying paper having a coating applied on the paper support or substrate thereof, said coating comprising naphthalenesulfonate formaldehyde condensate of the formula:



(wherein R is H, CH<sub>3</sub> or C<sub>2</sub>H<sub>5</sub>, M is Na, K, Li or NH<sub>4</sub>, and n is an integer of 1 to 20), said coating imparting low surface resistance properties to said support.

**10 Claims, No Drawings**

[56] **References Cited**

UNITED STATES PATENTS

|           |        |                |           |
|-----------|--------|----------------|-----------|
| 3,121,708 | 2/1964 | Engelmann..... | 117/155 L |
| 3,240,594 | 3/1966 | Cassiers.....  | 96/1.5    |
| 3,240,597 | 3/1966 | Fox .....      | 96/1.5    |

## ELECTROPHOTOGRAPHIC COPYING PAPER

## BACKGROUND OF THE INVENTION

## 1. Field of the Invention

This invention relates to electrophotographic copying paper having an electrically conductive paper support or substrate, and a method of making same. More particularly, this invention comprises treating the paper base or substrate of electrophotographic copying paper with naphthalenesulfonate formaldehyde condensate to impart low-resistance properties thereto.

## 2. Description of the Prior Art

Electrophotography is a well-known photographic reproduction technique utilizing the combined characteristics of photoconductivity and electrostatic phenomenon. It is, in principle, based on the theory of Xerography invented by C. F. Carlson.

Electrophotographic copying paper is prepared by applying on a low-resistance base or substrate a photoconductive powder dispersion or photoconductive sensitive layer comprising zinc oxide powder dispersed in a binder such as, for example, silicon resin or unsaturated polyester, so as to be capable of forming electrostatic latent images through the action of light. It is required that the surface resistance of the low-resistance base or substrate be within the range of from  $10^6$  to  $10^9$   $\Omega$  (ohms) when the relative humidity of the ambient atmosphere is from 20 to 90 percent. It is believed that if the surface resistance is outside that range, a good image cannot be obtained.

This invention has for its object to provide an improved electrophotographic copying paper in which the base or substrate has applied thereto a low resistance processing agent that can satisfy the above-mentioned requirements.

As processing agents for preparing conductive processed papers, there have been used heretofore anionic water-soluble polymers such as poly(vinylbenzyltrimethylammonium chloride) as disclosed in U.S. Pat. Nos. 3,620,828 and 3,011,918. More recently, oligostyrene-maleic anhydride copolymers have been used as more effective agents.

## SUMMARY OF THE INVENTION

According to the invention, there is provided an improved electrophotographic copying paper in which the base or substrate has applied thereto a coating of naphthalenesulfonate formaldehyde condensate of the formula:



(wherein R is H,  $\text{CH}_3$  or  $\text{C}_2\text{H}_5$ , M is Na, K, Li or  $\text{NH}_4$ , and n is an integer of from 1 to 20). The condensate is applied to the base or substrate in the form of an aqueous solution or aqueous dispersion thereof which is then dried so that the condensate is present on the base or substrate in the form of fine particles adhering to the surface of the base or substrate.

The naphthalenesulfonate formaldehyde condensate according to the present invention is applied in an amount of 0.1 to 10  $\text{g/m}^2$ , preferably 1 to 3  $\text{g/m}^2$ , calculated as the solids, based on the surface area treated of the paper base or substrate. The aqueous solution or dispersion of said condensate is usually applied by itself to the base paper, but if required, a known additive or additives which have been generally used heretofore, such as inorganic metal salts, surfactants, moisture absorbers or polyelectrolytes can be used in admixture with said condensate.

Various types of coaters such as roll coaters, sizing presses, knife coaters or bar coaters can be used for applying said aqueous solution or dispersion to the base paper.

In applying the naphthalenesulfonate formaldehyde condensate, it is usually desirable, as aforementioned, to apply it in the form of a water solution when said condensate is water-soluble or in the form of aqueous dispersion when said condensate is dispersed in water with the aid of a dispersant.

The conductive processed base paper obtained by applying to the base paper the processing agent of the present invention is low in surface electric resistance over a wide humidity range, and the electrophotographic copying paper produced by using such processed paper can produce high-quality images.

After processing the base paper or substrate with the processing agent, in accordance with this invention, a photoconductive layer or film is applied on top of the processing agent and adhered to the substrate to form the completed electrophotographic copying paper. The photoconductive layer comprises a dispersion of organic or inorganic photoconductive substance dispersed in a resinous binder having relatively high electrical resistivity. It is preferred to use photoconductive zinc oxide as the photoconductive substance. The binder resin can be selected from any of those suitable for preparing such photoconductive layers. It will be understood that the present invention does not relate to any discovery relating to the composition of the photoconductive layer. This can be selected from compositions suitable for this purpose. A detailed description thereof is believed to be unnecessary because suitable compositions are well known.

Among the naphthalenesulfonate formaldehyde condensates that can be used in the present invention are  $\alpha$ - or  $\beta$ -naphthalenesulfonate formaldehyde condensates in which R is H, or naphthalene sulfonate formaldehyde condensates in which R is an alkyl group with 1 to 2 carbon atoms, such as methyl or ethyl group, and the like. The preferred condensate is  $\beta$ -naphthalenesulfonate formaldehyde condensate. Another preference is for compounds in which n is from 4 to 12. These compounds, for example, the sodium salt of formaldehyde condensate of  $\beta$ -naphthalene sulfonic acid are known compounds. They can be synthesized in, for instance, the following way.

288 Grams (1 mol) of  $\beta$ -naphthalenesulfonic acid, 30 grams (0.3 mol) of 95 percent sulfuric acid and 48 grams of water are put into a four-necked flask. A substantial portion of the  $\beta$ -naphthalenesulfonic acid is dissolved at 80° to 85°C, and then 17.2 grams of an aqueous solution containing 35.8 wt. percent formaldehyde is added to the solution. While maintaining the mixture at 80° to 85°C, further amounts of 17.2 grams of said formaldehyde solution are added after 1, 2 and

3 hours, respectively, so that the total amount of formaldehyde solution added is 68.8 grams (0.82 mol). After the completion of the addition of formaldehyde solution, the mixture is heated to 95° to 100°C in 20 minutes and reacted at that temperature for a period of 7½ hours. Then, an aqueous solution of calcium carbonate is added to perform liming, and then sodium carbonate is added to the hot filtrate to form the sodium salt. The insoluble inorganic salts are filtered away, and the filtrate is evaporated to obtain the sodium salt of  $\beta$ -naphthalenesulfonic acid formaldehyde condensate ( $n=6$ ,  $R=H$ ,  $M=Na$ ).

The invention is further described by reference to the following illustrative examples.

#### EXAMPLE

Aqueous solutions of the respective low-resistance processing agents (conductive processing agent) listed in the following table were applied by a knife coater on one side of a commercial high-quality cellulosic fiber paper (weighing 70 g/m<sup>2</sup>) such that said agent was applied in amount of 2 g/m<sup>2</sup>, calculated as the solids, based on the treated area of the paper. After drying the treated paper under reduced pressure, specimens of the treated paper were placed in desiccators having 20 percent relative humidity (RH) and 60 percent relative humidity, respectively, and were allowed to stand therein for 24 hours. Thereafter, the specimens were taken out of said desiccators and their surface resistances were measured by using as measuring electrodes, Model RC-02 manufactured by Kawaguchi Denki Seisakujo. The results are shown in Table 1 below. The processing agents were used in the form of 30 wt. percent aqueous solutions.

35

Specimen Nos. 6 to 8 are comparison specimens employing different metal salts of the condensate. As is apparent from the table, the surface resistance characteristics of the treated base papers, under different humidity conditions, obtained from the specimens of the present invention are far better than those obtained from the comparison specimens.

It was also confirmed by hand touch that the processed papers prepared according to the present invention remain nonsticky even in a highly humid atmosphere.

Then, a zinc oxide — resin binder composed of a uniform mixture of 4 parts by weight of zinc oxide powder and 1 part by weight of resin binder (unsaturated polyester having an average molecular weight of 3,000) obtained by reacting 3,3-di(4- $\beta$ -hydroxypropoxyphenyl propane) with fumaric acid, was applied in an amount of 20 g/m<sup>2</sup> on the conductive processed papers (Specimen Nos. 1 to 5) according to the present invention to produce electrophotographic recording papers. The image-forming characteristics of the thus obtained recording papers were examined by testing them in a commercial electrophotographic copying machine. Vivid and clear images can be obtained with any of these recording papers.

#### Comparative Example

Conductive processed papers were prepared according to the same method and under the same conditions as in the above-described example by using two representative types of commercial conductive treating agents. The surface resistance of the thus obtained processed papers at 20 and 60% RH was measured. The results are shown in Table 2 below in comparison with

Table 1

| Specimen No.                      | Processing agent                                                              | Surface resistance of processed paper (ohms) |                      |
|-----------------------------------|-------------------------------------------------------------------------------|----------------------------------------------|----------------------|
|                                   |                                                                               | RH 20%                                       | RH 60%               |
| Examples of the Present Invention | 1 Sodium $\beta$ -naphthalenesulfonate formaldehyde condensate ( $n = 6$ )    | $7.0 \times 10^7$                            | $5.5 \times 10^7$    |
|                                   | 2 Ammonium $\beta$ -naphthalenesulfonate formaldehyde condensate ( $n = 6$ )  | $5.0 \times 10^7$                            | $3.8 \times 10^7$    |
|                                   | 3 Lithium $\beta$ -naphthalenesulfonate formaldehyde condensate ( $n = 6$ )   | $1.0 \times 10^8$                            | $8.9 \times 10^7$    |
|                                   | 4 Potassium $\beta$ -naphthalenesulfonate formaldehyde condensate ( $n = 6$ ) | $7.2 \times 10^7$                            | $6.5 \times 10^7$    |
|                                   | 5 Sodium $\beta$ -naphthalenesulfonate formaldehyde condensate ( $n = 10$ )   | $9.8 \times 10^7$                            | $5.5 \times 10^7$    |
| Comparative Examples              | 6 Magnesium $\beta$ -naphthalenesulfonate formaldehyde condensate ( $n = 6$ ) | $1.1 \times 10^{10}$                         | $8.7 \times 10^9$    |
|                                   | 7 Strontium $\beta$ -naphthalenesulfonate formaldehyde condensate ( $n = 6$ ) | $1.3 \times 10^{10}$                         | $8.0 \times 10^9$    |
|                                   | 8 Zinc $\beta$ -naphthalenesulfonate formaldehyde condensate ( $n = 6$ )      | $2.5 \times 10^{10}$                         | $8.0 \times 10^9$    |
|                                   | 9 Not treated                                                                 | $3.4 \times 10^{11}$                         | $1.3 \times 10^{11}$ |

In the above table, Specimen Nos. 1 to 5 are specimens prepared according to the present invention, whereas

the test results of Specimen No. 1 of the present invention.

Table 2

| Specimen No.         | Treating agent                                                             | Surface resistance of treated paper (ohms) |                   |
|----------------------|----------------------------------------------------------------------------|--------------------------------------------|-------------------|
|                      |                                                                            | RH 20 %                                    | RH 60 %           |
| Comparative Examples | 10 Poly(vinylbenzyltrimethylammonium chloride)*                            | $1.8 \times 10^8$                          | $1.2 \times 10^8$ |
|                      | 11 Poly(styrene sodium sulfonate)**                                        | $8.4 \times 10^7$                          | $6.0 \times 10^7$ |
| Present Invention    | 1 Sodium $\beta$ -naphthalenesulfonate formaldehyde condensate ( $n = 6$ ) | $7.0 \times 10^7$                          | $5.5 \times 10^7$ |

Note)

\* Tradename ECR 34 mfd. by Dow Chemical Co.

\*\* Tradename Oligo Z mfd. by Tomoegawa Paper Mfg. Co., Ltd.

These results show that the treating agents according to the present invention provide as good or better surface resistance characteristics than the best commercial products.

The embodiments of the invention in which an exclusive property or privilege is claimed are defined as follows:

1. In an electrophotographic copying paper comprising a support having on one surface thereof a photoconductive layer comprising a mixture of photoconductive substance and a film-forming resin binder, the improvement which comprises:

said surface of said support has applied thereon, underneath said photoconductive layer, a coating of naphthalenesulfonate formaldehyde condensate of the formula



wherein R is H, CH<sub>3</sub> or C<sub>2</sub>H<sub>5</sub>, M is Na, K, Li or NH<sub>4</sub>, and

n is an integer of 1 to 20,

in an amount effective to reduce the surface electrical resistance of said support to within the range of 10<sup>6</sup> to 10<sup>9</sup> ohms.

2. An electrophotographic copying paper according to claim 1, in which said coating is applied on said surface in an amount of from 0.1 to 10 g/m<sup>2</sup>, based on the area of said surface.

3. An electrophotographic copying paper according to claim 1, in which said coating is applied on said surface in an amount of from 1.0 to 3.0 g/m<sup>2</sup>, based on the area of said surface.

4. An electrophotographic copying material accord-

ing to claim 1, in which said support is paper made of cellulosic fibers.

5. An electrophotographic copying material according to claim 2, in which R is H and M is Na.

6. An electrophotographic copying material according to claim 1, in which n is from 4 to 12.

7. A method of producing paper processed to have a surface electrical resistance in the range of about 10<sup>6</sup> to about 10<sup>9</sup> ohms, which comprises applying to a surface of the paper a coating of an aqueous solution or dispersion of naphthalenesulfonate formaldehyde condensate of the formula



wherein R is H, CH<sub>3</sub> or C<sub>2</sub>H<sub>5</sub>, M is Na, K, Li or NH<sub>4</sub>, and

n is an integer of 1 to 20

and drying said coating.

8. A method according to claim 7, in which said coating is applied on said surface in an amount of from 0.1 to 10.0 g/m<sup>2</sup>, calculated as the solids, based on the area of said surface.

9. A method according to claim 7, in which said coating is applied on said surface in an amount of from 1.0 to 3.0 g/m<sup>2</sup>, calculated as the solids, based on the area of said surface.

10. A method according to claim 7, including the further step of applying on said surface having said dried coating thereon, a mixture of photoconductive substance and film-forming resin binder to form a photoconductive layer.

\* \* \* \* \*